

# UNITED STATES PATENT OFFICE.

JOHN M. NELSON, JR., OF SHERWOOD, MARYLAND.

## PROCESS OF PRESERVING WOOD.

937,008.

No Drawing.

Specification of Letters Patent. Patented Oct. 12, 1909.

Application filed July 1, 1908. Serial No. 441,513.

To all whom it may concern:

Be it known that I, JOHN M. NELSON, Jr., a citizen of the United States, and an employee of the Forest Service, Department of Agriculture, a legal resident of the State of Maryland, residing at Sherwood, county of Baltimore, Maryland, (whose post-office address is Forest Service, Department of Agriculture, Washington, District of Columbia,) have invented new and useful Improvements in the Process of the Treatment of Timber with Liquid Preservatives, and made application by petition of even date herewith, under the act of March 3, 1883, chapter 143, 22 Stat., 625, praying that Letters Patent therefor may be granted to me.

The invention herein described and claimed may be used by the Government of the United States or any of its officers or employees in the prosecution of work for the United States or by any person in the United States without the payment of any royalty thereon.

The following is a specification of the said invention:

This invention has relation to the process of treating timber with liquid preservatives such as creosote oil and zinc chlorid for the purpose of preventing decay. I do not, however, confine myself to the preservatives mentioned.

The object of the improved process is to secure a deeper penetration of the wood with a smaller amount of the preservative than is obtained by the methods commonly in use.

The process of treatment consists in immersing the wood in a first bath of suitable preservative or non-preservative liquid, which bath is above the temperature of boiling water. In this bath the wood becomes heated and the air and moisture contained within it are expanded and a portion of them driven out of the wood, the action extending to a depth which depends upon the degree of heat used and the time for which the timber is left in the bath. At the end of a sufficient time, the wood is freed from the unabsorbed portion of the preservative or non-preservative liquid of the first, or hot bath, and immediately immersed in a second bath of preservative liquid, which is at a temperature below that of boiling

water, or the wood is left in the preservative liquid of the first bath, which is cooled to a temperature below that of boiling water to 55 constitute the second bath. In either case the temperature of the wood becomes lowered in the second bath, and a partial vacuum is formed in the cells and other spaces within the wood by the contraction of the air and 60 other vapors which have previously been heated and expanded. The preservative liquid is therefore drawn into the wood, the amount which is so drawn in, and the depth to which it penetrates depending upon the 65 extent of the action which has been produced by the first, or hot bath, above described, and the length of time the wood is left in the second, or cold bath. The wood is then freed from the unabsorbed portion of the second, 70 or cool bath and again subjected to a third bath of preservative or non-preservative liquid, whose temperature is above the boiling point of water and preferably somewhat above the temperature of the first bath, care 75 being exercised, however, that the temperature be not high enough in either case to injure the strength of the wood, or the wood is left in the preservative liquid of the first and second baths which is raised to a tem- 80 perature like that described above for the third bath. The effect of this third, or final hot bath is that any given amount of preservative liquid which has been drawn into the wood is distributed through a deeper 85 zone, that is to say, a deeper penetration of wood is secured with a smaller amount of the preservative liquid than is possible with the use of the first two baths only, which has before been stated to be the object of this in- 90 vention.

The process embodied in this invention is applicable to the preservative treatment of timber with liquid preservatives in any manner, using closed cylinders, with or without pressure, or open tanks or vats. But it is especially adapted for use with what is known as the open-tank process. To explain it more specifically, therefore, I will describe its application to this process in 100 detail:

First, as applied to heavy timbers: The timber is first submerged in a preservative or non-preservative liquid in an open tank,

which is then heated to a temperature of about 220° F., constituting the first bath. This temperature is maintained for a period of about two hours. The temperature of 5 the preservative is then lowered, constituting the second bath, to 150° F., or until the timber has absorbed 5 pounds of the preservative per cubic foot, or such amount as may be necessary to obtain the desired penetration. The temperature of a preservative 10 or non-preservative is then raised to about 230° F., constituting the third bath, and is there held for a period of approximately 3 hours, when the timber, while still hot, is 15 taken out of the preservative in a treated condition.

Second, as applied to light timbers: The timber is submerged in a preservative or non-preservative liquid in an open tank, 20 which is heated, and thereafter cooled, to the same degrees of temperature and for the same periods of time as above described for heavy timbers; or, the timber may be transferred, at the end of the first hot bath period 25 to another tank containing cold preservative, constituting the second bath, until the desired impregnation is secured. It is then returned to the heated preservative or non-preservative liquid of the first bath, which 30 has, in the meantime, been raised to a temperature of about 230° F., constituting the third bath, and is there held for a period of three hours, at the end of which time the timber, while still hot, is taken out of the 35 preservative or non-preservative in a treated condition.

The essential feature of my invention is the successive immersion of wood in a preservative or non-preservative liquid heated 40 above the boiling point of water, then in preservative liquid at a temperature below the boiling point of water, and finally, again in preservative or non-preservative liquid heated above the boiling point of water and 45 preferably somewhat hotter than the liquid of the first immersion.

I have above illustrated the process as applied to the use of two separate and distinct tanks containing hot and cold liquids 50 respectively, or of a single tank in which the liquid is successively heated and cooled; but my invention may be applied with equal success with any other method of manipulating the liquids to obtain the desired end, as 55 well as with closed tanks or cylinders. When a single tank is used, the liquid may be cooled by artificial means if desired; or instead of cooling the liquid when the wood 60 has been immersed for a sufficient time in the first, or hot bath, this liquid may be drawn off and its place supplied by cold liquid, which in turn may again be replaced by hot.

In the processes above specified either a

preservative or a nonpreservative liquid may 65 be used in the first bath; in the second bath a preservative liquid must be used; in the third bath a preservative or a nonpreservative liquid may be used. The preservative liquids used in my process may consist of 70 such substances as creosote, crude petroleum, and oil tar or aqueous solutions of the following chemical salts;—zinc chlorid, sodium chlorid, magnesium chlorid, and copper sulfate. These liquids or materials may be 75 used alone or in combination. The nonpreservative liquids used in my process may consist of such substances as liquid asphalt, crude oil, and coal tar. My invention, however, is not limited to the use of any of the 80 preservative or nonpreservative liquids above enumerated; it includes the use of any preservative or nonpreservative liquid or liquids whatever in carrying out the process described and specified.

85

What I claim, and desire to secure by Letters Patent is:

1. The method of preventing deterioration or decay of timber, which consists in first subjecting the timber to a suitable bath 90 heated above the boiling point of water, second, lowering the temperature of the bath, third raising the temperature to a point above that of the initial bath, and, finally, removing the timber from the liquid and 95 allowing it to cool in the open air, substantially as specified.

2. The method of preventing the deterioration and decay of timber which consists in subjecting the timber to a suitable bath, heated to a temperature sufficient to expand and drive off a portion of the gas and moisture contained in the timber, then lowering the temperature of the bath sufficiently to permit the absorption of the required 105 amount of preservative into the timber, due to the contraction of the gases and moisture, then raising the temperature to a point, preferably slightly above that of the first bath in order that more of the gases and 110 moisture in the interior of the timber may be driven off, and finally submitting the timber to the action of the air, in order that the preservative in the exterior portions of the timber may be drawn farther into the 115 timber, due to the contraction caused by the cooling of the atmosphere.

3. The method of preserving timber and the like which consists in first subjecting the same to the action of a bath of a suitable 120 liquid heated to a temperature of over 100° C., then to a bath of a suitable preservative liquid at a lower temperature, then to the action of a bath of a suitable liquid at a temperature at least as high as the first bath, 125 substantially as described.

4. The method of preserving timber and the like which consists in first subjecting the

937,008

same to a bath of a suitable liquid at a temperature of over 100° C., then lowering the temperature to permit absorption, then again raising the temperature to disseminate the absorbed liquid, substantially as described.

In testimony whereof I affix my signature in the presence of the two subscribed wit-

nesses, this twenty-fifth day of April, 1908,  
at Washington, District of Columbia.

JOHN M. NELSON, JR.

Witnesses:

W. F. SHERFESSEE,  
CHAS. R. PIERCE.